

## UNITED STATES PATENT OFFICE

2,626,900

POLYPROPYLENE BENZENE SULFONATE  
DETERGENT COMPOSITIONS CON-  
TAINING TETRASODIUM PYROPHOS-  
PHATESamuel A. Russell, III, Chicago, Ill., assignor to  
Allied Chemical & Dye Corporation, New York,  
N. Y., a corporation of New YorkNo Drawing. Application January 29, 1949,  
Serial No. 73,659

3 Claims. (Cl. 252—138)

1

This invention relates to the manufacture of detergent compositions. It is particularly concerned with improvements in detergent compositions of the alkyl benzene sulfonate type.

The manufacture of alkyl benzene sulfonate detergents normally involves alkylation of benzene, sulfonation of the alkylated benzene, and neutralization of the sulfonic acid product. Neutralized products obtained in this manner may be used without further treatment or with only removal of water, and in this condition are effective and efficient detergent compositions. Such compositions normally contain between 30% and 45% of alkyl benzene sodium sulfonate, and between 55% and 70% of sodium sulfate. In some cases the mixtures are treated for removal of the sodium sulfate to produce alkyl benzene sodium sulfonates substantially free of inorganic salts.

For the manufacture of detergents of the above types benzene has been alkylated by several methods and by several types of alkylating compounds. For example, benzene has been condensed with chlorinated kerosene fractions in the presence of an aluminum chloride condensing agent. Benzene has been condensed also with olefins from various sources, employing aluminum chloride, sulfuric acid, or other suitable condensing agent. Olefins employed for this alkylation have been obtained by dehydration of alcohols, by cracking of petroleum products, and by polymerization processes. Thus olefins obtained by polymerization of propylene, butylene, isobutylene and amylene have been proposed.

Regardless of the source, the most suitable alkylating compounds are those providing alkyl groups containing between 9 and 18 carbon atoms.

Alkyl benzene sulfonate detergents have been marketed alone and also in admixture with other detergent materials, among which may be mentioned the phosphates, such as trisodium phosphate and sodium triphosphate. Experimental tests have demonstrated that while such phosphates may improve some commercial alkyl aromatic sulfonate detergents slightly, the improvement is not great. Moreover, tetrasodium pyrophosphate does not always promote the detergent action of such alkyl benzene sulfonates, as illustrated by its effect, in a normal hard water, upon a commercially available detergent comprising alkyl benzene sulfonates derived from chlorinated kerosene and upon such a detergent derived from polypropylene fractions having an average molecular carbon content of 12 carbon atoms, as shown in Table II below.

2

Contrary to expectation from the results observed when tetrasodium pyrophosphate is employed with such detergents, it has been found, in accordance with the present invention, that the addition of tetrasodium pyrophosphate has a decidedly beneficial effect upon "polypropylene" benzene sulfonate detergents having an average of 13 to 15 carbon atoms in the "polypropylene" radicals and containing a substantial proportion of pentamers among the "polypropylene" radicals. This discovery has led to the production of superior detergent compositions and furthermore has permitted utilizing for the production of such compositions substantially less expensive starting materials.

The compositions of my invention comprise such "polypropylene" benzene sodium sulfonates in which the "polypropylene" radicals contain an average of 13 to 15 carbon atoms, and in addition to the sulfonate, between 1 and 3 parts of sodium sulfate and between 1 and 4 parts of tetrasodium pyrophosphate for each part by weight of the sulfonate, these proportions being determined on the dry basis. The products of the invention when employed in water at a concentration of  $\frac{1}{4}\%$  provide a pH between 9 and 10.4.

Polypropylene fractions of about 200° to 270° C. boiling range boiling for the most part between 210° and 260° C. have the required average molecular carbon content and contain pentapropylene as the major component. Such polypropylene fractions, suitable for preparing the products of the invention, are available commercially. They are normally produced by the superatmospheric polymerization of propylene in the presence of a Friedel-Crafts type catalyst, such as boron trifluoride or aluminum chloride. These commercial polypropylene fractions may be employed as such for the alkylation of benzene, and the resulting polypropylene benzene, upon sulfonation and neutralization, yields polypropylene benzene sulfonate suitable for use in my invention.

The alkylation may be effected by means of any suitable alkylation catalyst such as sulfuric acid, boron trifluoride, hydrogen fluoride or aluminum chloride, commonly designated Friedel-Crafts type catalysts.

The following example illustrates the manufacture of a detergent within the purview of the invention:

172 parts of 95%  $H_2SO_4$  is mixed with 42 parts of benzene at 10° to 20° C. 65 parts of polypropylene, distilling at normal atmospheric pres-

sure from 200° to 250° C., is added rapidly to the benzene sulfuric acid mixture while the temperature of the mixture is maintained below 20° C. by cooling. After all of the polypropylene is added, which normally should be accomplished in a period between 10 minutes and one hour, the mixture is stirred for 1½ hours at a temperature not above 30° C. The product is then allowed to stratify and the heavy  $H_2SO_4$  layer is withdrawn. The alkylate which remains is neutralized with aqueous sodium carbonate solution

woven cotton fabric soiled with a suspension of graphite in lubricating oil and cottonseed oil. The proportion of soil removed was determined photometrically.

When the above detergents were mixed with tetrasodium pyrophosphate and tested at a total detergent concentration of 0.25%, employing an identical test, substantially different results were obtained. The following table shows the variation of these results with varying proportions of tetrasodium pyrophosphate.

Table II

|                                                                                 | 100% Detergent | Detergent-TSPP Ratio |       |       |       |       |       |
|---------------------------------------------------------------------------------|----------------|----------------------|-------|-------|-------|-------|-------|
|                                                                                 |                | 90-10                | 80-20 | 70-30 | 60-40 | 50-50 | 40-60 |
| Polypropylene ( $C_{14}$ ) Benzene Sodium Sulfonate Detergent (62% $Na_2SO_4$ ) | 17             | 22                   | 29    | 39    | 48    | 51    | 44    |
| Polypropylene ( $C_{12}$ ) Benzene Sodium Sulfonate Detergent (62% $Na_2SO_4$ ) | 40             | 30                   | 23    | —     | 34    | —     | —     |
| Keryl Benzene Sodium Sulfonate Detergent (62% $Na_2SO_4$ )                      | 38             | 29                   | 23    | 35    | 35    | 38    | —     |

and stripped with steam to remove unreacted benzene. After removal of the benzene the alkylate is again permitted to stratify and the water and sodium sulfate and sodium carbonate are drawn off. The remaining alkylate is then dried with anhydrous calcium chloride and separated from this drying agent.

To effect sulfonation of the alkylate 50 parts of the alkylate is cooled to between 10° and 20° C. and 100 parts of 20% oleum is added while the mixture is stirred vigorously with cooling to maintain the temperature below 20° C. When all of the oleum has been added, agitation is continued until the end of 4 hours from the time of starting the addition of oleum, the temperature being maintained during this period below 30° C. The sulfonation mixture is then introduced gradually into 285 parts of aqueous 25% NaOH solution at a temperature of about 45° C. The pH of the slurry is adjusted finally to approximately 7 by the addition of sulfuric acid and the slurry is then dried. Drying may be effected by means of a drum drier or a spray drier at 110° C. The dry product contains about 38% of alkyl benzene sodium sulfonate and 62% of sodium sulfate. Upon application of the process on a large scale, the content of alkyl benzene sodium sulfonate and sodium sulfate may vary 5% above or below these values.

The following tables show the results of launderometer tests of this detergent product in comparison with a commercial product made from chlorinated kerosene and a polypropylene benzene sulfonate having an average of only 12 carbon atoms in the "polypropylene" radicals. These tests were made employing water having a hardness corresponding to 300 parts per million of calcium carbonate.

Table I

| Detergent Concentration, Percent | Polypropylene Benzene Sulfonate |          | Keryl Benzene Sulfonate |
|----------------------------------|---------------------------------|----------|-------------------------|
|                                  | $C_{14}$                        | $C_{12}$ |                         |
| 0.1                              | 12                              | 9        | 17                      |
| 0.25                             | 18                              | 40       | 38                      |
| 0.5                              | 29                              | 40       | 38                      |

The values in this table represent the percentage of soil removed in a standard test involving a

divergence of results in Table II, 100% detergent, and Table I, 0.25% concentration, represent deviations within the limits of experimental error.

From Table II it is apparent that in these tests, in the absence of tetrasodium pyrophosphate, the keryl benzene sulfonate detergent gave better soil removal than the  $C_{14}$  polypropylene benzene sulfonate detergent, but upon addition of tetrasodium pyrophosphate gave poorer and poorer results, and in no case gave better results than in the absence of the tetrasodium pyrophosphate, whereas the  $C_{14}$  polypropylene benzene sulfonate upon addition of tetrasodium pyrophosphate gave better and better results until at a 50-50 ratio this detergent was substantially superior to any of the mixtures of keryl benzene sulfonate as well as to this product without the tetrasodium pyrophosphate. The product from 12 carbon atom (average) polypropylene resembled the keryl product in its behavior and all its mixtures with TSPP tested were inferior to the 100% detergent product.

I claim:

1. A detergent composition consisting essentially of "polypropylene" benzene sodium sulfonate, in which the "polypropylene" radicals contain an average of between 13 and 15 carbon atoms and comprise a substantial proportion of "pentapropylene" radicals, and for about each one part by weight of polypropylene benzene sodium sulfonate (dry basis), between 1 and 3 parts of sodium sulfate and between  $\frac{1}{3}$  and 4 parts of tetrasodium pyrophosphate.

2. A detergent composition consisting essentially of "polypropylene" benzene sodium sulfonate, in which the "polypropylene" radicals correspond substantially entirely to olefins boiling between 200° and 270° C., comprise as the major component "pentapropylene" radicals and contain an average of between 13 and 15 carbon atoms, and for about each one part by weight of polypropylene benzene sodium sulfonate (dry basis), between 1.3 and 2 parts of sodium sulfate and between 1 and 3 parts of tetrasodium pyrophosphate.

3. A detergent composition consisting essentially of "polypropylene" benzene sodium sulfonate, in which the "polypropylene" radicals correspond substantially entirely to olefins boiling between 200° and 270° C. and predominantly between 210°

and 260° C., comprise as the major component "pentapropylene" radicals and contain an average of between 13 and 15 carbon atoms, and for about each one part by weight of polypropylene benzene sodium sulfonate (dry basis) about 1½ parts of sodium sulfate, and for each part of total sulfonate and sulfate about ⅔ to 1 part of tetra-sodium pyrophosphate.

SAMUEL A. RUSSELL, III.

10

REFERENCES CITED

The following references are of record in the file of this patent:

UNITED STATES PATENTS

| Number      | Name     | Date          |
|-------------|----------|---------------|
| 2,330,922   | Riegler  | Oct. 5, 1943  |
| 2,351,559   | Treffier | June 13, 1944 |
| 5 2,394,320 | McGhie   | Feb. 5, 1946  |
| 2,396,278   | Lind     | Mar. 12, 1946 |
| 2,477,382   | Lewis    | July 26, 1949 |
| 2,477,383   | Lewis    | July 26, 1949 |
| 2,486,922   | Strain   | Nov. 1, 1949  |

OTHER REFERENCES

Oil and Soap, vol. 23, 1946, page 105.